

O. C. WINESTOCK.  
INDURATED POROUS MATERIAL AND PROCESS OF FORMING SAME.  
APPLICATION FILED AUG. 16, 1919.  
1,377,241. Patented May 10, 1921.



Fig. 1.



Fig. 2.

Inventor  
Fig. 3. Otto C. Winestock

By

George Ramsey  
his Attorney

# UNITED STATES PATENT OFFICE.

OTTO C. WINESTOCK, OF PERKINSVILLE, VERMONT, ASSIGNOR TO WALTER W. SLACK,  
OF SPRINGFIELD, VERMONT.

## INDURATED POROUS MATERIAL AND PROCESS OF FORMING SAME.

1,377,241.

Specification of Letters Patent. Patented May 10, 1921.

Application filed August 16, 1919. Serial No. 318,051.

*To all whom it may concern:*

Be it known that I, OTTO C. WINESTOCK, a citizen of the United States, residing at Perkinsville, in the county of Windsor, 5 State of Vermont, have invented certain new and useful Improvements in Indurated Porous Materials and Processes of Forming Same, of which the following is a specification.

10 This invention relates broadly to the indurating of fibrous materials, and specifically to the indurating of shoe lasts. It comprises a novel process for the induration of fibrous materials, and a wooden shoe last embodying a structure produced by the practice of such process.

Among its several objects and advantages, the invention includes the provision of a new and advantageous process of indurating 20 fibrous material whereby occluded liquids and gases, such as water, wood sap, air, carbon dioxid, etc., may be removed from the porosities of fibrous materials such as wood, and the porosities permanently filled with a 25 tenacious elastic material, so as to effectively eliminate the capillary, bibulous and hydroscopic qualities of the wood, increase its homogeneity and density, and preserve its structural form.

30 Another object of the invention is the provision of a novel method of the sort specified which is effective in securing the intended results in a very short period of time.

35 Another object of the invention is the provision of a process having the attributes above mentioned and which may be effectively practised upon articles of considerable size or bulk, such as blocks of wood 40 having such mass or thickness as not to be ordinarily penetrable or permeable by liquid.

45 A further object of the invention is the provision of a process having the attributes above specified and which may be practised at very low cost and with entire safety to the materials upon which it is used, the plant in which it is utilized, and the individuals by whom it is actually carried on.

50 A still further object of the invention is an article of manufacture consisting of a shoe last formed of wood, having its porosities filled with a stable tenacious elastic material and possessing certain distinctive

advantages and novel features hereinafter 55 to be more particularly pointed out.

Other objects of the invention will be obvious from the following specification and claims, and the drawings forming a part of the specification or will be pointed out specifically therein.

Heretofore the induration of fibrous materials such as wood, leather, and the like, have been successful only within limits quite strictly imposed by the size of the 65 articles to be indurated and the cost of the process used. Induration of thin materials, such as fabrics, leather, thin wood, and the like, has been practised with success in varying degrees. The induration of soft or 70 porous wooden articles, such as blocks or piling, of spruce or pine, with creosote preparations has been developed to a fairly satisfactory commercial degree so far as 75 surface preservation is concerned. The induration of thick pieces of hard, close grained wood, however, has not been successfully accomplished in a way that is practicable commercially. This has been due to the fact that those skilled in the art have 80 been unable to secure a sufficient penetration of the material by the indurating fluid by any commercially practical method. Various expedients have been resorted to to increase the extent of penetration or 85 permeation. One condition heretofore regarded as prerequisite has been that the wood be thoroughly dried and seasoned before being subjected to the indurating process.

The predrying or seasoning requires several 90 months of careful handling in dry houses, and is attended with a considerable loss of material from checking and cracking in the seasoning process. Accordingly it is extremely expensive. Efforts have been made 95 to increase the penetration of the indurating fluid by the use of pressure. This has

proven unsatisfactory, both from the danger and cost incident to utilizing pressure, and due also to the fact that as the pressure influence is but temporary, indurating fluid forced into the porosities of the wood under pressure is subsequently expelled with greater or less rapidity by the expansion of the occluded gases within the wood, when the exterior pressure is removed, or the generation of further pressure in the wood by the decomposition of organic matter therein.

Certain experimenters have endeavored to secure increased penetration by forming artificial channels into the wood for the passage of the indurating fluid by punching or 5 boring holes, or by forcing apart the wood fibers. The treatment of the material in this fashion is necessarily objectionable when it is intended for uses which require 10 homogeneity of the structure, and particularly a smooth, well finished and resistant surface.

By the employment of the process comprised in my present invention, I am enabled to eliminate the disadvantages pertaining 15 to the methods heretofore employed, and also to secure certain distinct advantages not contemplated by others who have been active in the art. For example, I am enabled to take blocks freshly cut from green 20 logs and, by my process, completely expel the gases and liquids occluded in the pores of the material, and fill all such porosities with a stable elastic material which will prevent reabsorption of gases or liquids by 25 the wood, all in the course of a single treatment within a very short time.

While my process is suitable for use upon a great variety of articles I will describe it as applied to the indurating of wooden 30 blocks for the manufacture of shoe lasts, and the drawing shows an article of that kind for the purpose of illustrating the process.

In the drawing, Figure 1 represents a side elevation of a last block;

35 Fig. 2 a section on the line 2—2 of Fig. 1 and Fig. 3 a diagrammatic illustration of an apparatus for practising the process.

As is well known in the art, in the manufacture of shoes, lasts made of wood are employed upon which the shoes are shaped and built. These articles must possess certain 40 characteristics in order to fit them for their use. In the first place, the material must be suitably workable so that the last may be 45 accurately formed to the proper size and shape. Furthermore, the material must be of such quality as to have a minimum susceptibility to weather or atmospheric changes, in order that they may retain their 50 shape and their size accurately. In present practice it is customary to keep the lasts, when not in use, in a dry-house wherein the temperature and moisture content of the air are carefully regulated for uniformity. 55 This necessitates the removal of the lasts from the dry-house every morning for use in the factory and also their replacement in the dry-house at the end of the day. A further quality which such articles must possess is that of good finish, density and firmness. They must have a good smooth dry 60 finish in order to contribute to the proper forming and smoothing of the inside of the shoe, and they must be dry in order that 65 they will not affect the material of the shoe

or gather foreign matter, and in order that they may be manipulated easily in removal from the shoe. They must be firm and of good density because of the handling to which they are subjected in the manufacture 70 of the shoes so that they will hold the lasting tacks but will not be made soft or porous or pulpy by the punctures thereof. The life of a last is limited both by the usage to which it is subjected and by change in 75 styles of foot wear. The average last is good for use in about eighty shoes. Due to the necessity of replacement, there is an annual requirement of something in excess of three million blocks for this use. The 80 present customary practice is to cut the blocks, intended for manufacture into shoe lasts, from hard close grained and homogeneous timber such as hard maple, and then subject the blocks to a course of drying and 85 seasoning extending over a period of several months.

In the manufacture of indurated blocks suitable for shoe lasts by the use of my improved process, I take the blocks of wood, 90 just either dried or as they are cut from the logs, and while yet unseasoned and having more or less moisture content, and preferably, though not necessarily, trim them down to approximately the size of the lasts 95 intended to be formed from them,—such a block is designated by the numeral 1 in the drawing. This shaping is simply for the purpose of removing all possible excess material and thereby reducing handling 100 costs, waste of indurating composition, and unnecessary expenditure of time in processing. Such trimming of the blocks will also serve to discover checks or cracks or other faults in the material not discernible in the 105 original block. The blocks are then provided with a venting channel 2. This venting channel is preferably formed by boring a hole in the material so as to leave a clear and unobstructed channel, said hole being 110 formed in a portion of the block where it will not interfere with the use of the finished article. It is important that this venting channel extend deeply into the block, and it is desirable that it penetrate the block in its 115 most massive portion. Preferably the channel is bored transversely of the grain of the wood so that it will intersect as many as possible of the natural veins, channels and rays of the wood structure. It is not necessary, however, that the venting channel be formed across the grain, as it is effective 120 also when formed parallel with the grain. In the illustration I have shown the venting channel as extending deeply into the last block at the thickest part thereof, which is in a portion corresponding to the arch and instep of the foot, and in which location it will not interfere with any of the uses to 125 which the last is put. The channel may 130

be formed in other locations, however. So prepared, the green blocks are ready for subjection to the processing with the indurating compound.

- 5 The indurating compound comprises a substantially saturated solution of vulcanized rubber in ordinary kerosene. The approximate proportion is 1 pound of rubber to 6 quarts of kerosene, but the exact proportion depends upon the quality of rubber used. If it is comparatively new and live rubber, a smaller proportion will give the composition the proper body than if the rubber is old rubber. The rubber utilized 10 may be in the form of scrap rubber such as old vehicle tires, inner tubes and the like. The solution is obtained by raising the kerosene to a temperature sufficiently high to melt the rubber, and then mixing in the rubber in small pieces until the liquid has taken up all that it can hold. Any solids and foreign matter contained in the rubber scrap will be precipitated or floated and are readily strained out of the liquid, leaving 15 the latter clean and free from slime. In some cases it may be desirable to add a very small amount of amyl acetate, which contributes somewhat to hastening the dissolution of the rubber, and also to disguising any disagreeable odor of the compound.

The indurating compound having been thus prepared, it is placed in a suitable vessel or kettle 4 and the blocks, prepared as above described, deposited in it, preferably while it is cold. The liquid with the blocks is then raised to a temperature of from 140° F. to 198° F. and maintained thereat for a period suitable to permit the permeation of the material of the blocks by the indurating liquid. In the case of wet green blocks of hard maple weighing in the neighborhood of 30 ounces and suitably vented as above described, I have found that the treatment with the liquor at the temperature above mentioned for about twenty-four hours has been effective. During the treatment of the blocks in the liquid, it appears that the following takes place:

The heat transmitted to the wood through the liquor is effective to expand the same somewhat and increases its bibulous capacity, thereby facilitating the rapid penetration of the liquid into the porosities of the wood. This penetration is contributed to, no doubt, also by the hydrostatic pressure of the liquor upon the outer surface of the blocks. The penetration of the hot liquor into the porosities of the wood conveys the heat to the occluded gases and entrained liquids therein, causing an expansion of the former, which is effective to force the liquids out of the channels in which they are entrained. Their evacuation is accommodated by the vent which provides a channel 65 of egress from the interior of the block, so

that there is no opportunity given for development of a pressure within the porosities of the wood effective to resist the ingress of the indurating liquid. This action is evidenced by the fact that during the treatment of the blocks there is a very active discharge from the mouth of the vent channel, perceptible as a forcible jet of bubbles spouting out of the channel into the liquid. This discharge from the vent evidently comprises the occluded and entrained gases and liquids, and other gases generated in the porosities of the wood by the heat. Part of the water thus expelled from the wood passes off as vapor, and part of it settles to the bottom of the receptacle, being immiscible with the indurating fluid. This discharge from the venting channel gradually decreases in volume during the period that the blocks are left in the liquor. When the discharge ceases to be perceptible, it may be taken as indicative of the fact that the originally occluded and entrained gases and liquids have been displaced by the indurating fluid. Such a condition in the blocks 70 having been reached, the source of heat to the vessel is cut off so that the liquor and the blocks therein will be allowed to cool gradually. These blocks are left in the liquid 75 for a sufficient time to permit them 80 reaching approximately atmospheric temperature, and even longer if they are dense. With blocks of the sort above described, I have found that three days in the liquid 85 after the heating have given excellent results. During this cooling the blocks contract to 90 approximately their original size. The blocks are then removed from the indurating liquid and permitted to dry in the atmosphere. This they do quite rapidly, all 95 excess liquid on the surface being evaporated, leaving the material dry and clean. The kerosene in the liquid which has penetrated the wood gradually evaporates, leaving 100 the porosities filled with the rubber. 105

Blocks in this condition may then be shaped and dressed down to the form of the finished lasts, without further treatment or seasoning.

If desired, the lasts may be re-treated after 115 being finished, the course of procedure above described being repeated. This will contribute to the production of the hard smooth finished surface on the finished last.

As a means of heightening the finish, and 120 producing a polish and case-finish, in the treatment of finished lasts there may be added to the liquid an amount of pure linseed oil equaling about  $\frac{1}{16}$  of the total volume. The linseed oil is added to the rubber-kerosene composition just after the latter has been made and clarified, and while it is still hot. This small quantity of linseed oil oxidizes on the surface finish on the lasts, heightening the finish and producing a very 125 130

- high polish of handsome color. This obviates the use of the expensive wax now used to surface the lasts, and, therefore, the added expense of applying and polishing same.
- 5 It is found that in the utilization of this process the material in addition to being impregnated by the indurating fluid, is completely deprived of the free gaseous and fluid content of the porosities and cells.
- 10 I have specified above that a temperature of about 198° F. is effective in the treatment of the blocks. This, of course, admits of variation. The point to be observed is that as high a temperature as possible is desirable, excepting that the temperature must not be permitted to reach the point where it will cause expansion of the occluded gases and liquids greatly in excess of their rate of egress, as such development of pressure 15 within the wood structure forces the fibers apart and produces checking. Blocks subjected to this process and indurated by the composition specified show no effects from subsequent atmospheric changes or wettings 20 or dryings, even under extreme conditions which would not be encountered in practical use of shoe lasts. This may be explained from the fact that the occluded and entrained gases and liquids are displaced, and 25 from the particular nature of the indurating material. In the indurating fluid the kerosene constitutes a solvent and vehicle in which the rubber is handled for transmission into the porosities of the wood. Kerosene forms an excellent vehicle in this composition and process due to the facts that it forms an effective solvent and carrier for the rubber and, while sufficiently volatile to evaporate under atmospheric temperatures 30 leaving the rubber *in situ*, it is not so volatile as to be dangerous in the practice of the process with the use of an open flame for heating the containing receptacle. For this reason also there is no expensive loss by 35 evaporation of the liquid under the increased temperature during the practice of the process, and the indurating liquid thereby maintains a desirable fluidity which enables its rapid penetration into the wood. Furthermore, it is inexpensive, and does not require special equipment for preservation or safekeeping. The rubber, which is entrained in the porosities and natural channels of the 40 wood under the influence of the heat, becomes occluded therein upon the cooling of the blocks and forms a tenacious elastic filler completely occupying and closing such porosities, coating the cell structures and thereby insulating them and inhibiting 45 changes in their hygroscopic condition. The rubber, being tenacious and coherent, forms a highly stable filler, so that it is not displaced by changes of temperature, and its composition is not broken down. Hence, it 50 does not exude from the wood. Being elastic, and being deposited in the porosities of the wood when the latter are expanded by heat, it accommodates the expansion and contraction of the wood structure without being itself displaced, and without permitting the porosities to become open or unoccupied. In these particulars it differs quite essentially from various indurating compositions which include grease or other unstable constituents. In the use of prior compositions of this kind I have observed that the material, under different influences, breaks down, so that various of its contents, such as the greases, are exuded from the surface of the wood. Not only does this render 55 the surface sticky and place the article temporarily out of use, but it also indicates the progressive loss of the filler. Inasmuch as it is the filler which is depended upon to inhibit the susceptibility of the wood to moisture and atmospheric changes, it will be seen that the loss of the filler means the reduction of the ability of the material to maintain its size and form in the presence of different moisture and atmospheric conditions. My 60 indurating composition, especially when applied by the process described, has the further advantage, particularly in contrast to compositions which include non-volatile greases, of providing a binder for the cellular structure of the wood which is effective to preserve its structural form and increase its density and homogeneity. Compositions heretofore employed and containing greases have the effect of softening the wood structure, rendering the cellular and fibular structure more loose and pliable, and thereby making the article soft and, to a degree, pulpy. It will be seen, therefore, that an article indurated with my improved composition 65 will be distinctly superior to those treated with the prior compositions in any uses wherein hardness and homogeneity of the structure and smoothness and durability of surface are important. For this reason 70 shoe lasts having a structure characterized by the inclusion of my improved indurating composition are of distinct superiority. Not only are they immune to the contemplated moisture and atmospheric changes, but they 75 are also very durable and wear resisting, susceptible of hard and high finish, capable of being easily and accurately worked and formed, and are thoroughly stable in the retention of the indurating material. 80
- Having thus described my invention, what I claim is:
1. The process of indurating porous material which comprises providing the material with an unobstructed venting channel 85 extending into the interior thereof, then treating the material in a bath of hot indurating liquid containing oxidizable material and permitting the egress of occluded fluid from the porosities of the material through 90

- the venting channel, permitting the material to partially cool in the indurating fluid, and then subjecting the material to oxidizing influences.
- 5    2. The process of indurating porous material which comprises providing the material with an unobstructed venting channel extending into the interior thereof, then placing the material in a bath of hot indurating 10 liquid containing rubber and an oxidizable material, and permitting the egress of occluded fluid from the porosities of the material to become cool in the indurating fluid, and then removing the material from the indurating fluid and exposing it to atmosphere.
- 15
3. As an article of manufacture, a shoe last comprised of wood with the porosities thereof filled with a stable tenacious elastic material. 20
4. As an article of manufacture, a shoe last of wood with the porosities thereof filled with rubber.
5. As an article of manufacture, a shoe last of wood indurated with a stable elastic 25 vegetable gum.
6. As an article of manufacture, a shoe last comprised of wood with the porosities thereof filled with a stable tenacious elastic material and having an oxidized surface 30 film.

OTTO C. WINESTOCK.